

1,207,726.

C. V. EADES.  
WATERPROOFING.  
APPLICATION FILED MAR. 28, 1914.

Patented Dec. 12, 1916.



Witnessed,  
D. J. Mann,  
Joyce M. Lutz

Inventor,  
Charles V. Eades

By Frank L. Belknap,  
7444.

# UNITED STATES PATENT OFFICE.

CHARLES V. EADES, OF CHICAGO, ILLINOIS, ASSIGNOR TO STANDARD ASPHALT & RUBBER COMPANY, OF CHICAGO, ILLINOIS, A CORPORATION OF NEW JERSEY.

## WATERPROOFING.

1,207,726.

Specification of Letters Patent. Patented Dec. 12, 1916.

Application filed March 28, 1914. Serial No. 828,104.

To all whom it may concern:

Be it known that I, CHARLES V. EADES, a citizen of the United States, residing in the city of Chicago, county of Cook, and State of Illinois, have invented certain new and useful Improvements in Waterproofing, of which the following is a specification.

My invention relates to improvements in water-proofing and has among its salient objects to provide a construction which is adapted for roofing such as concrete roofs and roofs of bridges, viaducts and the like; to provide a construction in which the upper or wearing surface of the water-proofing is secured to the foundation by an elastic bond or membrane which allows for contraction or expansion to obviate cracking or breaking of the other members of the water-proofing; to provide a construction in which the membrane becomes an integral mass bonded to the foundation and to the protection or upper coating if any; to provide a construction which has as an essential feature a pair of flexible fabric members united by a binder of bituminous putty; to provide a construction which when used for roofs of railway bridges or viaducts is peculiarly adapted to deaden noise and absorb shocks while at the same time affording a firm and substantial base for the ballast and track; and in general to provide an improved construction of the character referred to.

The invention consists in the matters hereinafter described and more particularly pointed out in the appended claims.

In the drawings, Figure 1 is a sectional view with parts broken away showing the invention as applied to a concrete roof; Fig. 2 is an enlarged sectional detail of the portion of the membrane; Fig. 3 is a vertical sectional view showing the invention in use on the roof of a railway viaduct or bridge.

Referring first to the construction shown in Figs. 1 and 2, 1 designates as a whole the concrete roof, although the material of which the roof is made is not important. This concrete foundation is first covered with a paint or primer coat 2 of liquid asphaltic paint which intimately mixes with the upper surface of the foundation. On this paint coating is next put a mop or binder coat 3 of solid asphalt which is heated until liquid and then poured on the primer coat 2 to the desired thickness. It is to be noted that the primer coat is a

liquid one when cold while the mop coat is not liquid when it is heated above its melting point. The melting point of the mop coat may be about 180° F., although this will vary as conditions may require. Both the paint coat and the mop coat may consist of blown oil asphaltic compounds and the mop coat particularly should be water-proof and not subject to extremes of weather. To this mop coat while still hot is applied a flexible fabric 4 such as burlap which sticks and adheres to the mop coat. Above the fabric 4 is a second similar fabric 6, the two being separated from each other and united by means of an asphaltic bond 5 which is or may be of bituminous putty, consisting essentially of a mixture of lime dust and asphalt. The melting point of the bond may be about 165° F., although this too will vary widely with conditions. Upon the upper face of the fabric 6 is placed a second mop coat 7, similar to the mop coat 3 heretofore described. On top of this mop coat 7 is placed a fabric covering 8 which may consist of felt saturated with asphalt. The various coats heretofore described form a membrane, the members of which are so connected and bonded together with each other as to form a substantially unitary structure, which itself is bonded to the foundation whether of concrete or other material.

In Fig. 3 is shown the application of the invention to a railway bridge or viaduct. In this instance, there is the same foundation 1, upon which is formed the membrane heretofore described, designated as a whole A. Upon this membrane is supported the rock or other ballast 9 between which and the top covering of the membrane is interposed a mastic 10 which assists in forming a shock absorber. This mastic coating 10 is preferably formed of bituminous concrete. The melting point of this mastic coating may be 450° F., although this will vary and hence it is essential to have the top asphalt saturated felt coating 8 interposed between the mastic and the mop coat and bituminous putty. This is obvious for the reason that the melting point of the mastic is so high that when applied hot the mop coat and bituminous putty would melt and bring the fabric through the mastic if there was no protection between such as the covering 8. The bituminous bond 5 is flexible even below zero and materially assists in the matter of

expansion and contraction and deadens sound, particularly when used beneath railway ballast. The bond 5 forms in effect a bituminous cushion bonding the two flexible fabrics 4 and 6. The mop coats not only waterproof the outer surface of the fabrics, but also serve to bind the same to the foundation, and to the felt covering 8. The object of using the fabric is to prevent the membrane from breaking through when subjected to severe torsional strains or severe shocks. The primer or paint coat cleans the foundation and closes the pores and recesses of the upper surfaces of the same and makes an anchorage for the subsequent coatings. The mop coat, for instance, will not stick to the concrete except when the primer coat is used. The second mop coat prevents deterioration of the fabric and binds the same to the adjacent coatings. The membrane as a whole forms a substantially integral member as will be obvious from the foregoing description.

The invention is not limited to the details of construction shown except as set forth in the appended claims.

I claim as my invention:

1. In a waterproofing, the combination with a foundation, of a paint coat on the upper surface of said foundation, a pair of asphaltic mop coats, flexible fabrics between the mop coats and a bituminous cushion between said fabrics, said cushion and coats uniting with each other to form a substantially unitary structure.

2. In a waterproofing, the combination with a rigid foundation, of a pair of bituminous saturated fabrics on said foundation, a relatively thick bituminous cement bond coat interposed between the fabrics and bituminous mop coats above and below the fabrics.

CHARLES V. EADES.

Witnesses:

JOYCE M. LUTZ,  
F. L. BELKNAP.